

# United States Patent Office

2,699,413

Patented Jan. 11, 1955

1

2,699,413

## COATING COMPOSITION FOR CONTAINERS AND CLOSURES THEREFOR

George William Seagren, Pittsburgh, and George Lawrence Reyman, Sewickley, Pa., assignors to Stoner-Mudge, Inc., Pittsburgh, Pa., a corporation of Pennsylvania

No Drawing. Application May 20, 1952,  
Serial No. 288,998

8 Claims. (Cl. 148—31.5)

This invention relates to the art of resinous coatings for containers for foods and beverages and closures therefor, in particular containers and closures made of sheet steel or black plate as it is commonly called.

Tin plate has been conventionally employed but the lighter coating weights of tin now commonly used do not always provide sufficient protection for certain foods and beverages and resinous coatings have been applied to tin plate to provide the necessary protection.

The requirements of such resinous coatings are very severe. Those requirements include adhesion and the flexibility necessary to maintain that adhesion during and after the deformation encountered in fabrication of the coated plate, e. g. into can ends and screw caps plus the inertness necessary to avoid imparting any undesirable flavor or toxic ingredient to the food or beverage contents of the container and to avoid any substantial impairment of the resinous film by the action of the container contents or water or steam at the high temperatures encountered in processing the containers and their contents.

The following are some of the more important tests which have been developed to measure the requirements of resinous can and closure coatings or enamels:

Dry adhesion

Process wet adhesion

Process blush resistance

Process blistering resistance

Process spotting resistance

Chemical and organic-solvent resistance

Underfilm corrosion resistance to oxygen-containing acid foods

Stain resistance to sulphur-bearing products

Flexibility and fabrication (dry and after processing)

Flavor and odor freedom

Because of the increasing scarcity and unreliability of tin sources, the art for many years has tried to develop satisfactory coatings for direct application to the surface of sheet steel or black plate, thus eliminating the need for the surface coating of tin, as it is present on tin plate.

It has been found, however, that the elimination of tin with its accompanying electrochemical protective action on iron creates an additional problem because the conventional types of coating well-known in the art, which meet the above requirements when applied to tin plate, are not adequate when applied directly to plain sheet steel or black plate because of the susceptibility of plain steel to corrosion, particularly under the coating, when exposed to steam and hot water, and the lack of stability of coatings in direct contact with a surface of plain steel. Therefore a coating for direct application to iron or steel must have additional properties to compensate for the loss in electrochemical protection which results from the elimination of tin.

The more discriminatory tests for judging whether a coating (i. e. lacquer or enamel) is satisfactory as applied directly to sheet steel or black plate for use in the manufacture of cans and closures for food and beverage products are as follows: The "oxygenated spinach" test, which measures the resistance of the coating to peeling and loosening and also the underfilm corrosion resistance of the metal; the "meat staining" test which measures the stain resistance to sulfur-bearing products; the "process blush" test which measures the resistance of the coating to steam or water at elevated temperatures such as 250° F.; the "solvent resistance" test which gives an indication of the insolubility and chemical inertness of the coating. These tests of course are run only on coatings which show

2

satisfactory fabrication properties, which is a prime requirement for a can or closure enamel.

These tests are described briefly as follows:

The "oxygenated spinach" test: This is an accelerated test indicative of the resistance of the coating to foods, particularly the mildly acid ones, and demonstrates in a few days rather than many months of normal shelf-aging, the effectiveness of the coating in preventing the attack of the steel substrate by these food chemicals, shows the resistance of the coating to "blush" or whitening on contact with the water in the food product, and shows the retention of flexibility and good adhesion upon exposure of the coating to the food, heat and pressure to which the coated article is subjected during the processing operation. In this test a can, the inside surface of which is provided with the coating to be tested, is filled with spinach, evacuated, and the air replaced by pure oxygen. The container thereupon is sealed and processed in steam at 240° F. for 60 minutes. After allowing to stand for several days the container is opened and the coated metal examined for deterioration and attack by the food mixture. If the coating is not "processable" the coating may have turned white ("blushed") or have lost adhesion or both. If the coating has not protected the steel substrate from underfilm corrosion, numerous areas or the total area will have corroded or rusted. If the coating protects the steel substrate from under-film corrosion there will be no rust or corroded areas. An estimate of the resistance of the coating in the oxygenated spinach test is made by visually observing and determining the percentage area of coated metal surface unattacked. A perfect rating of 100 is obtained when none of the coated surface shows attack. A rating of 90 signifies that 90% of the coated area shows no signs of corrosion. A minimum rating of 75 on certain products will be acceptable to the metal can or closure manufacturing industry, though naturally as high a rating as possible is preferred.

The "meat staining" test: This test demonstrates the protection the coating affords the steel substrate against staining by sulfur-bearing bodies present in food products, such staining being due to the formation of iron sulfides or other iron compounds. In this test, coated sheet steel panels are placed in a synthetic meat mixture comprised usually of edible oils, organic acids, carbohydrates, proteins, esters, salts and moisture and the whole subjected to steam processing (autoclaving) for two hours at 250° F. At the conclusion of the processing, the panels are removed, cleaned of adhering food product, and rated visually for degree of staining or blackening. A perfect rating of 100 means no blackening of the coated steel while a rating of 50 indicates slight darkening, and a rating of 0 complete blackening. Depending upon the product packaged and other considerations, a minimum rating of 50 may be acceptable to the container manufacturing industry, though naturally as high a rating as possible is preferred.

The "solvent resistance" test: In this test the effect of methyl ethyl ketone (MEK) on the coating baked on a sheet steel substrate is determined and an indication of the insolubility, chemical inertness and degree of thermosetting of the organic coating is obtained. In this test the baked coating on a steel substrate is rubbed ten times with a cloth saturated with methyl ethyl ketone. At the end of the manipulation the coating is visually examined for softening or solution by the ketone solvent. A perfect rating of 100 indicates that the coating is neither softened nor dissolved by the methyl ethyl ketone and is to that extent chemically inert. A rating of 50 means that the coating is softened by the solvent and is not as chemically inert or thermoset. A zero rating indicates the coating to be dissolved by the solvent and thus to possess a low order of insolubility, chemical inertness and thermoset properties.

The term "process blush resistance" is well known and relates to a test wherein the coated material is subjected in an autoclave to steam at about 15 lbs. pressure for about 30 minutes. The perfect rating of 100 means that the coating does not lose gloss, transparency and does not whiten or "blush," while a rating of 0 means that the coating has lost gloss completely and/or becomes whitened

or opaque. A rating of 70 or less indicates unsatisfactory performance.

It is also necessary that the coating shall behave satisfactorily when subjected to the "fabrication" test. In that test a steel panel is provided with the coating and after the baking operation is drawn and curled into the shape necessary for a can end or is formed into a screw closure by imparting a thread, curl and knurl, using appropriate dies and other machinery. A satisfactory coating shows no substantial separation of the coating from the steel substrate as a result of these forming operations. The fabrication behavior of the coating is made readily apparent by immersing the coated can end or closure in an acidified copper sulfate solution for about 1 minute.

A principal object of the invention is to provide a lacquer or enamel coating for cans or closures used for food products, beverages and other packaged products, where that lacquer or enamel is applied as a single coat directly to steel or black plate, in the form of sheets or in the form of partially or completely fabricated containers or closure.

A further object is to provide such a lacquer or enamel coating which meets all the mentioned tests including the more important oxygenated spinach, meat staining, process blush and solvent resistance tests.

A further object is to provide a coating material which may be applied directly to steel or black plate (preferably a lighter coating weight than when used as a single enamel coat) to serve as a "primer" or base coat on the metal, which is subsequently to be over-coated with one or more additional coats of lacquer, enamel, ink or coating of a chemical type different from that of the present invention.

In accordance with the invention, a resinous composition consisting essentially of three components is provided, those components being (a) a particular kind of polyepoxide resin, (b) a particular kind of phenolic resin, and (c) from 5-20% of phosphoric acid ( $H_3PO_4$ ) based on the total weight of resinous components (a) and (b).

Polyepoxide resins are well known as such. They are polyethers containing recurring hydroxy-ether groups and having terminal epoxide groups. They are commonly made by reacting a compound having two reactive hydrogen atoms, e. g. a polyhydric phenol or a polyhydric alcohol, with epichlorhydrin or a dichlorhydrin. Bis-phenol is frequently used as the compound supplying reactive hydrogen atoms. When that is reacted with epichlorhydrin the general formula of the resulting polyepoxide resin is



where  $n$  varies with molecular weight from a value of 4 to a value of 24.

The properties of the polyepoxide resins vary with variations of the molecular size. The average molecular weight is readily determined by ebulliometry or cryoscopy.

In this invention polyepoxide resins are used which are polyglycidyl ethers of dihydric phenols having a molecular weight of 1500 to 7200.

A typical procedure, to illustrate the above definition, as described in the art for making such polyglycidyl ethers (polyepoxide resins) is as follows:

A relatively low molecular weight product (polyglycidyl ether 1) may be made by reacting 1 mol of bisphenol in 1 liter of water containing in excess of 2 mols of NaOH and 2.05 mols of epichlorhydrin which is then dissolved in that solution by addition thereto at 40° C. with stirring. An exothermic reaction ensues which raises the temperature of the reaction mixture to 65° C. in about thirty minutes. As soon as the reaction subsides, heat is applied to bring the mixture to the boiling point, in about thirty minutes, and the mixture is then refluxed for an additional sixty minutes. An unstable emulsion of the resin in water is obtained. The oily resinous layer is allowed to settle and is washed by decantation to remove salt, excess NaOH, epichlorhydrin, and other impurities. Upon subsequent vacuum dehydration, a balsamic solid resin is obtained with a melting point of about 45° C. and a molecular weight of about 500 to 600.

The higher molecular weight polyepoxide resins required in this invention are then obtained by heating the polyglycidyl ether 1 produced as described with additional bisphenol, with or without an alkali catalyst, for several

hours at 200° C. The following table shows the proportions of reactants which may be used to give the higher molecular weight polyglycidyl ethers or polyepoxide resin:

|    | Grams polyglycidyl ether 1 | Grams bisphenol | M. W. of Product |
|----|----------------------------|-----------------|------------------|
| 10 | 100                        | 50              | 1,800-1,900      |
|    | 100                        | 35              | 3,000-4,000      |
|    | 100                        | 30              | 5,000-7,200      |

In the above typical procedure, instead of bis-phenol, dihydric phenols in general may be used, for example, resorcinol or hydroquinone.

In accordance with the present invention the solids of the coating composition consist essentially of two resin components, resin A and resin B, and a proportion of orthophosphoric acid of 5 to 20% by weight of the total resin solids. Resin A is a polyepoxide resin as above defined. Resin B is a particular kind of phenolic resin compatible with polyepoxide resin A and is an organic solvent-soluble alkali condensed condensation product of formaldehyde and a phenol of the group consisting of a 2,3 dialkyl phenol, 2,5 dialkyl phenol, 3,4 dialkyl phenol, 3,5 dialkyl phenol, 2 monoalkyl phenol, and 4 monoalkyl phenol, where the alkyl group has from one to five carbon atoms. Also commercial mixtures composed principally of any two or more of the above substituted phenols may be used, for example, certain selected phenolic mixtures composed principally of the members of the group described, such as "mixed xylenols," "cresylic acid," "cresols" and "butyl phenols" of commerce where the substituents on the benzene nucleus are alkyl groups.

A typical procedure, to illustrate the above definition, for making a phenolic resin (resin B) suitable for this invention is as follows:

Charge into a resin reactor, 610 parts of mixed xylenols, 546 parts of aqueous 37% formaldehyde and 61 parts of aqueous 28% ammonia; heat with agitation to about 82° C. in a period of one hour and hold with continuing agitation at this temperature for an additional period of one hour; stop the heating and agitation and decant the water layer; distill under about 24 inches of vacuum at a temperature of about 93° C. for about 3 hours to remove moisture and unreacted ingredients. This yields a hard friable resin, which is suitable for this invention.



The two resins are used in the ratio by weight of from 50% resin A and 50% resin B to 80% resin A and 20% resin B.

The resins and phosphoric acid are dissolved in volatile solvents to provide a liquid coating composition having a proportion of non-volatile coating solids of about 25 to 40% by weight, and having a viscosity of 25 to 100 seconds as measured in a #4 Ford Cup at 80° F.

Epoxide resin A is not per se thermosetting and phenolic resin B per se may or may not be thermosetting. However, the combination of the three components, epoxide resin, phenolic resin, and phosphoric acid, provides a thermosetting composition and the liquid coating compound when baked at 300° F. to 400° F. as a coating on sheet steel, yields an infusible, relatively insoluble, thermoset coating, which meets all the required tests, and in particular the tests for underfilm corrosion which are especially important for can coatings on sheet steel and which are herein designated as the "oxygenated spinach," "meat staining," "process blush," "fabrication" and "solvent resistance" tests.

Purely for purposes of illustration the following example is submitted, showing a preferred liquid coating composition in accordance with the invention:

|                      | Solids          |                   |
|----------------------|-----------------|-------------------|
|                      | Parts by weight | Percent by weight |
| Resin A.....         | 70              | 61                |
| Resin B.....         | 30              | 26                |
| Phosphoric Acid..... | 15              | 13                |
|                      | 115             | 100               |

|                      | Percent by weight |
|----------------------|-------------------|
| Ethoxyglycol acetate | 26                |
| Isophorone           | 17                |
| n-Butanol            | 14                |
| Xylool               | 43                |
|                      | 100               |

The solids in this particular example are dissolved in the solvent in the proportion of 34% by weight of solids and 66% by weight of solvent and the resulting solution is applied to steel sheet by roller-coating to yield a film weight (of the dry film) of 4 mgms. per square inch and baked at 375° for 10 minutes. The resulting coating when subjected to the oxygenated spinach test gave a rating of 90.

While this example represents a typical solvent composition suitable for roller-coating application, it is understood that other active solvents and compatible diluents may also be used in place of those mentioned above, as required to adjust such properties as the flow-out rate of the wet coating, and the rate or speed of dry, so that the coating may be suitable for varying speeds of roller-coating application or application by other means such as spraying, dipping, "slushing" or brushing.

The importance of all three components, (a) epoxide resin A, (b) phenolic resin B, and (c) phosphoric acid, in obtaining a coating composition which meets the requirements of a satisfactory can and closure enamel is shown by the data in Tables I and II below.

Table I

| Code Letter | Epoxide Resin                     | Pheno-lic Resin | H <sub>3</sub> PO <sub>4</sub> | Metal                    | Film Wt., Mg./Sq. In. | Bake          |
|-------------|-----------------------------------|-----------------|--------------------------------|--------------------------|-----------------------|---------------|
| A           | 80                                | 20              | 15                             | Steel                    | 3.9                   | 10' @ 375° F. |
| B           | 80                                | 20              | 0                              | do                       | 3.6                   | Do.           |
| C           | 80                                | 0               | 15                             | do                       | 3.9                   | Do.           |
| D           | 80                                | 0               | 0                              | do                       | 3.8                   | Do.           |
| E           | 0                                 | 20              | 15                             | do                       | 4.9                   | Do.           |
| F           | 0                                 | 20              | 0                              | do                       | 3.7                   | Do.           |
| G           | 0                                 | 0               | 15                             | do                       | 0.25                  | Do.           |
| H           | 0                                 | 0               | 0                              | do                       |                       |               |
| J           | Oleo-Resinous Sanitary "C" Enamel |                 |                                | do                       | 3.9                   | 15' @ 400° F. |
| K           | do                                |                 |                                | Electro-lytic Tin-plate. | 3.9                   | Do.           |

SHOWING RESULTS OF TESTS ON THE COMPOSITIONS IDENTIFIED BY THE CODE LETTERS

| Code Letter | Oxygen-ated Spinach <sup>1</sup> | Meat Stain-ing <sup>2</sup> | Steam Process Blush <sup>3</sup> | Solvent Resist-ance <sup>4</sup> | Fabrication <sup>5</sup>      |
|-------------|----------------------------------|-----------------------------|----------------------------------|----------------------------------|-------------------------------|
| A           | 85                               | 100                         | 100                              | 100                              | Satisfactory.                 |
| B           | 25                               | 10                          | 100                              | 0                                | Do.                           |
| C           | 60                               | 90                          | 40                               | 100                              | Do.                           |
| D           | 5                                | 0                           | 0                                | 0                                | Do.                           |
| E           | 0                                | 0                           | 30                               | 100                              | Unsatisfactory (brittle). Do. |
| F           | 25                               | 80                          | 100                              | 100                              |                               |
| G           | 0                                | 0                           |                                  |                                  |                               |
| H           | 0                                | 0                           |                                  |                                  |                               |
| J           | 10                               | 0                           | 100                              | 40                               | Satisfactory.                 |
| K           | 90                               | 50                          | 100                              | 20                               | Do.                           |

<sup>1</sup> Processed 60 minutes @ 240° F. Stored 4 days at room temperature. Rating indicates percent coating remaining. 100=perfect; 0=complete failure.

<sup>2</sup> Strips processed 2 hours @ 250° F., in meat mixture. Examined when cool. Rating indicates degree of staining. 100=no staining; 0=complete staining.

<sup>3</sup> Action of steam at 15 lbs. pressure. A rating of less than 70 shows unsatisfactory performance.

<sup>4</sup> Rating indicates degree of softening after 10 rubs with MEK soaked rag. 100=no softening; 0=complete solution or removal.

<sup>5</sup> Can ends drawn and curled and behavior of lacquer on the fabrication test noted as satisfactory or unsatisfactory.

The compositions indicated by code letters A to F, inc. of the above data (Table I) were deposited from the same solvent mixture as given in the foregoing example, and baked under the same baking conditions. The epoxide resin of the compositions indicated by the code letters A-D, inc. was the same and was a polyepoxide polyglycidyl ether of bisphenol having a molecular weight of 5000-6000. The phenolic resin of the compositions

indicated by code letters A, B, E, and F was the same and was a condensation product of formaldehyde and mixed xylenols condensed to an alcohol soluble condition in the presence of an alkali. The figures indicating proportions of the various components mean parts by weight. In the case of code letters J and K, the same oleoresinous enamel was applied in both instances, in one case to steel and in the other case to tinplate; the solvent in this enamel is a mixture of conventionally employed liquid hydrocarbons; solvents of this type, while suitable and economical for use in oleoresinous enamels, are entirely unsuited for use in the compositions of codes A to F; neither would the solvent mixture used in the latter mentioned be suited for use in the oleoresinous enamel. Solvents are selected primarily for their ability to dissolve the solid constituents of the enamel, and once evaporated (as for example by baking) do not further influence the final baked film properties.

Referring to Table I, the different compositions are designated by the code letters A-G, with H representing untreated uncoated steel, and J and K used as "control" examples.

The composition of code A embodies the present invention and contains all three essential components of the solids of the coating composition, i. e. polyepoxide resin, phenolic resin, in the proportion of 80 parts polyepoxide and 20 parts phenolic resin by weight and 15 parts phosphoric acid. It provides satisfactory performance on all five important tests.

The composition of code B contains only two of the essential components of the present invention, that is, polyepoxide resin and phenolic resin in the proportion of 80 parts epoxide resin and 20 parts phenolic resin by weight, and no phosphoric acid. While satisfactory on the fabrication and the steam process blush tests, it is unsatisfactory on the oxygenated spinach, meat staining and solvent resistance tests.

The composition of code C shows the properties obtained when only the epoxide resin and phosphoric acid are used (80 parts of the former to 15 parts of the latter). No phenolic resin is present in this composition. While satisfactory for fabrication and for solvent resistance, it is slightly inferior in meat staining and grossly inferior in oxygenated spinach and steam process blush, to the composition containing all three components.

The composition of code D shows the results obtained for steel coated solely with the epoxide resin without the effect of the other two essential components of this invention, namely, the phenolic resin and phosphoric acid. It is satisfactory only in fabrication and is completely deficient in the four other properties requisite for a satisfactory can coating.

The composition of code E shows the effects on steel when it is coated with a composition containing only phenolic resin and phosphoric acid components in the ratio of 20 parts of the former to 15 parts of the latter. This composition has no polyepoxide resin present. This composition while possessing satisfactory solvent resistance properties, is grossly deficient in the other four principal properties required, including fabrication.

The composition of code F describes the properties obtained for steel coated with a composition containing solely the phenolic resin component of this invention, without any polyepoxide resin and phosphoric acid. While satisfactory for steam process blush and solvent resistance, this composition does not yield preferred meat staining resistance, fails on fabrication and is deficient in oxygenated spinach resistance.

Code G shows the results for steel that has been coated only with phosphoric acid. Since there is no organic film, steam process blush, solvent resistance and fabrication tests are inapplicable but it is completely unsatisfactory for oxygenated spinach and meat staining. Code H shows the properties of untreated uncoated steel when subjected to the appropriate tests. The same remarks apply as to code G.

In codes J and K, the compositions illustrate the results obtained by using a conventional oleoresinous sanitary can and closure enamel on steel (code J) and on tinplate (code K). This oleoresinous enamel, comprising a heat-bodied unsaturated vegetable oil and an unsaturated hydrocarbon resin is typical of enamels widely used today as coatings for tin plate. When applied to tin plate, it satisfactorily passes the oxygenated spinach, steam process blush and fabrication tests herein described,

as shown by code K, but when applied to steel as shown in code J, it is satisfactory only on steam process blush and fabrication tests and is completely unsatisfactory on the other three principal tests.

The data of the above Table I shows the necessity of using all three of the essential components—polyepoxide resin, phenolic resin and phosphoric acid—to obtain a composition which provides a coating that satisfactorily passes the principal test requirements as described in the specification when applied directly to sheet steel.

A comparison of the example of code A with code K shows that the composition of this invention provides a coating when applied directly to sheet steel which is even superior to the conventional oleoresinous coating on tin plate, particularly with respect to meat staining and solvent resistance.

The examples of codes B to G, where omission of one or two of the essential components occurs, show that the resulting compositions each lack one or more of the properties necessary to qualify the composition as an acceptable coating for containers and closures made from sheet steel for food and other products where the coating is applied directly to the steel surface.

Table II

## EPOXIDE RESIN PLUS PHENOLIC RESIN PLUS PHOSPHORIC ACID

| Parts<br>Epoxide<br>Resin | Parts<br>Phenolic<br>Resin | Parts<br>Phosphoric<br>Acid | Oxygenated<br>Spinach<br>Rating |
|---------------------------|----------------------------|-----------------------------|---------------------------------|
| 80                        | 20                         | 0                           | 25                              |
| 80                        | 20                         | 5                           | 75                              |
| 80                        | 20                         | 10                          | 80                              |
| 80                        | 20                         | 15                          | 85                              |
| 80                        | 20                         | 20                          | 80                              |
| 80                        | 20                         | 25                          | 60                              |
| 70                        | 30                         | 0                           | 30                              |
| 70                        | 30                         | 5                           | 80                              |
| 70                        | 30                         | 10                          | 85                              |
| 70                        | 30                         | 15                          | 90                              |
| 70                        | 30                         | 20                          | 85                              |
| 70                        | 30                         | 25                          | 65                              |

The above data (Table II) shows the compositions (in parts by weight) of coatings deposited on sheet steel from the same solvent and under the same baking conditions and at the same coating weight, the solvent being a mixed solvent composed of ethoxy-glycol acetate 26% by weight, isophorone 17% by weight, n-butanol 14% by weight, xylol 43% by weight. The baking time was 10 minutes at 375° F., and the coating weight was 4 milligrams of dry film-forming composition per square inch of sheet steel. The epoxide resin was the same in each of the above listed compositions and was a polyepoxide polyglycidyl ether of bisphenol having a molecular weight of 5000 to 6000. The phenolic resin was also the same in each of the said compositions and was a condensation product of formaldehyde and "mixed xylenols" condensed to an alcohol soluble condition in the presence of an alkali.

The values in Table II show that proportions of phosphoric acid from 5 to 20% by weight of the total weight of phenolic and epoxide resins give results, as measured by the "oxygenated spinach" test much superior to those obtained by proportions of phosphoric acid beyond the stated range, as used with proportions of epoxide resin to phenolic resin varying from 70% of epoxide resin and 30% of phenolic resin to 80% epoxide resin and 20% of phenolic resin and it has been found that substantially the same results are obtained with compositions where the proportions of epoxide to phenolic resin extends down to and including 50% of epoxide resin and 50% of phenolic resin.

Although the examples given herein illustrate clear (undyed and unpigmented) resinous films, applied by roller-coating to flat sheets of steel baked and subsequently fabricated into container ends, bodies and other parts and closures, it is understood that the scope of the invention also includes the addition of dyes, pigments, colorants and fillers to the liquid composition; also that with or without changes in the composition of the solvent portion of the liquid coating, the coating may be applied by any convenient means in addition to roller coating, such as by dipping, spraying, knifing, flushing, "slushing," wiping or brushing; also that although con-

tainers and closures made of sheet steel are usually coated and baked in flat sheets prior to any fabrication, the coating of this invention may also be applied to the sheet steel article that is, the container or closure, and baked thereon after the article has been partially or completely fabricated from the uncoated sheet stock.

What is claimed is:

1. A liquid coating composition adapted for direct application to sheet steel in the manufacture of containers and closures therefor consisting essentially of a resinous composition dissolved in a volatile organic solvent, said resinous composition being composed essentially of two resins, resin A and resin B, and from 5 to 20% by weight of orthophosphoric acid based on the total weight of said resins, resin A being a polyepoxide polyglycidyl ether of bisphenol having a molecular weight of 1500 to 7200, and resin B being an alkali catalyzed condensation product of formaldehyde and a phenol reactant of the group consisting of 2,3 dialkyl phenol, 2,5 dialkyl phenol, 3,4 dialkyl phenol, 3,5 dialkyl phenol, 2 monoalkyl phenol, 4 monoalkyl phenol, and mixtures thereof, where the alkyl group has from one to five carbon atoms, condensed to the organic solvent-soluble condition, the proportion by weight of resin A to resin B varying from 50% resin A and 50% resin B to 80% resin A and 20% resin B, and the proportion by weight of said resinous composition in said liquid coating composition varying from 25 to 40%.

2. A liquid coating composition adapted for direct application to sheet steel in the manufacture of containers and closures therefor consisting essentially of a resinous composition dissolved in a volatile organic solvent, said resinous composition being composed essentially of two resins, resin A and resin B, and 15% by weight of orthophosphoric acid based on the total weight of said resins, resin A being a polyepoxide polyglycidyl ether of bisphenol having a molecular weight of 1500 to 7200, and resin B being an alkali catalyzed condensation product of formaldehyde and a phenol reactant of the group consisting of 2,3 dialkyl phenol, 2,5 dialkyl phenol, 3,4 dialkyl phenol, 3,5 dialkyl phenol, 2 monoalkyl phenol, 4 monoalkyl phenol, and mixtures thereof, where the alkyl group has from one to five carbon atoms, condensed to the organic solvent-soluble condition, the proportion by weight of resin A to resin B varying from 70% of resin A and 30% of resin B, and the proportion by weight of said resinous composition in said liquid coating composition being about 34%.

3. A coated sheet steel article adapted for the manufacture of containers and closures therefor, said sheet having on at least one of its surfaces a baked-on coating of a resinous complex initially composed essentially of resin A and resin B and orthophosphoric acid, said coating resulting from the application to said steel surface of a coating of said resinous complex in an organic solvent-soluble, thermosetting condition and containing resins A and B in the proportion of from 50% by weight of resin A and 50% by weight of resin B to 80% by weight of resin A and 20% by weight of resin B, and from 5 to 20% by weight of orthophosphoric acid based on the combined amount of resins A and B, and thereafter heating said coated sheet to 350°-400° F. and converting said resinous complex to the thermoset condition, resin A in said soluble thermosetting resinous complex being a polyepoxide polyglycidyl ether of bisphenol having a molecular weight of 1500 to 7200, and resin B in said soluble thermosetting complex being an alkali catalyzed condensation product of formaldehyde and a phenol reactant of the group consisting of 2,3 dialkyl phenol, 2,5 dialkyl phenol, 3,4 dialkyl phenol, 3,5 dialkyl phenol, 2 monoalkyl phenol, 4 monoalkyl phenol, and mixtures thereof, where the alkyl group has from one to five carbon atoms, condensed to the organic solvent-soluble stage.

4. A coated sheet steel article adapted for the manufacture of containers and closures therefor, said sheet having on at least one of its surfaces a baked-on coating of a resinous complex initially composed essentially of resin A and resin B and orthophosphoric acid, said coating resulting from the application to said steel surface of a solution of said resinous complex in an organic solvent-soluble thermosetting condition and containing resins A and B in the proportion of 70% by weight of resin A and 30% by weight of resin B, and 15% by weight of orthophosphoric acid based on the combined amount

of resins A and B, and thereafter heating said coated sheet to 350°-400° F. and converting said resinous complex to the thermoset condition, resin A in said organic solvent-soluble, thermosetting resinous complex being a polyepoxide polyglycidyl ether of bisphenol having a molecular weight of 1500 to 7200, and resin B in said organic solvent-soluble thermosetting complex being an alkali catalyzed condensation product of formaldehyde and a phenol reactant of the group consisting of 2,3 dialkyl phenol, 2,5 dialkyl phenol, 3,4 dialkyl phenol, 3,5 dialkyl phenol, 2 monoalkyl phenol, 4 monoalkyl phenol, and mixtures thereof, where the alkyl group has from one to five carbon atoms, condensed to the organic solvent-soluble stage.

5. A liquid coating composition adapted for direct application to sheet steel in the manufacture of containers and closures therefor, consisting essentially of a resinous composition dissolved in a volatile organic solvent, said resinous composition being composed essentially of two resins, resin A and resin B and from 5 to 20% by weight of orthophosphoric acid based on the weight of said resins, resin A being a polyepoxide polyglycidyl ether of a dihydric phenol having a molecular weight of 1500-7200 and resin B being an alkali catalyzed condensation product of formaldehyde and a phenol reactant of the group consisting of 2,3 dialkyl phenol, 2,5 dialkyl phenol, 3,4 dialkyl phenol, 3,5 dialkyl phenol, 2 monoalkyl phenol, 4 monoalkyl phenol, and mixtures thereof, where the alkyl group has from one to five carbon atoms, condensed to the organic solvent-soluble condition, the proportions by weight of resin A to resin B varying from 50% resin A and 50% resin B to 80% resin A and 20% resin B, and the proportion by weight of said composition in said liquid coating varying from 25-40%.

6. A liquid coating composition adapted for direct application to sheet steel in the manufacture of containers and closures therefor, consisting essentially of a resinous composition dissolved in a volatile organic solvent, said resinous composition being composed essentially of two resins, resin A and resin B, and 15% by weight of orthophosphoric acid based on the total weight of said resins, resin A being a polyepoxide polyglycidyl ether of a dihydric phenol having a molecular weight of 1500-7200, and resin B being an alkali catalyzed condensation product of formaldehyde and a phenol reactant of the group consisting of 2,3 dialkyl phenol, 2,5 dialkyl phenol, 3,4 dialkyl phenol, 3,5 dialkyl phenol, 2 monoalkyl phenol, 4 monoalkyl phenol, and mixtures thereof, where the alkyl group has from one to five carbon atoms, condensed to the organic solvent-soluble condition, the proportion by weight of resin A to resin B being 70% of resin A and 30% of resin B, and the proportion by weight of said resinous composition in said liquid coating composition being about 34%.

7. A coated sheet steel article adapted for the manufacture of containers and closures therefor, said sheet

having on at least one of its surfaces a baked-on coating of a resinous complex initially composed essentially of resin A and resin B and orthophosphoric acid, said coating resulting from the application to said steel surface

5 ing resulting from the application to said steel surface of a solution of said resinous complex in an organic solvent-soluble, thermosetting condition and containing resins A and B in the proportions of from 50% by weight of resin A and 50% by weight of resin B.

10 resin A and 50% by weight of resin B to 80% by weight of resin A and 20% by weight of resin B, and from 5-20% by weight of orthophosphoric acid based on the combined amount of resins A and B, and thereafter heating said coated sheet to 350°-400° F. and converting said resinous complex to the thermoset condition, resin A in said soluble thermosetting resinous complex being

15 A in said soluble thermosetting resinous complex being a polyepoxide polyglycidyl ether of a dihydric phenol having a molecular weight of 1500-7200 and resin B in said soluble thermosetting complex being an alkali catalyzed condensation product of formaldehyde and a phenol reactant of the group consisting of 2,3-dihydro-

phenol reactant of the group consisting of 2,3 dialkyl phenol, 2,5 dialkyl phenol, 3,4 dialkyl phenol, 3,5 dialkyl phenol, 2 monoalkyl phenol, 4 monoalkyl phenol, and mixtures thereof, where the alkyl group has from one to five carbon atoms, condensed to the organic solvent-soluble stage.

25 8. A coated sheet steel article adapted for the manufacture of containers and closures therefor, said sheet having on at least one of its surfaces a baked on coating of a resinous complex initially composed essentially of resin A and resin B and orthophosphoric acid, said

30 coating resulting from the application to said steel surface of a solution of said resinous complex in an organic solvent-soluble thermosetting condition, and containing resins A and B in the proportion of 70% by weight of resin A and 30% by weight of resin B and 15% by

35 weight of orthophosphoric acid based on the combined amount of resins A and B, and thereafter heating said coated sheet to 350°-400° F. and converting said resinous complex to the thermoset condition, resin A is acid an-

40 complex to the thermoset condition, resin A in said organic solvent-soluble thermosetting resinous complex being a polyepoxide polyglycidyl ether of a dihydric phenol having a molecular weight of 1500-7200, and resin B in said organic solvent-soluble thermosetting complex being an alkylene oxide, the alkylene oxide being

an alkali catalyzed condensation product of formaldehyde and a phenol reactant of the group consisting of 2,3 dialkyl phenol, 2,5 dialkyl phenol, 3,4 dialkyl phenol, 3,5 dialkyl phenol, 2 monoalkyl phenol, 4 monoalkyl phenol, and mixtures thereof, where the alkyl group has from one to five carbon atoms, condensed to the organic

**References Cited in the file of this patent**

UNITED STATES PATENTS

- |    |           |                       |                |
|----|-----------|-----------------------|----------------|
| 55 | 2,296,070 | Thompson et al. ----- | Sept. 15, 1942 |
|    | 2,324,078 | Gray et al. -----     | July 13, 1943  |
|    | 2,521,911 | Greenlee -----        | Sept. 12, 1950 |